

E. L. WATROUS.

METHOD OF METAL PLATING.

APPLICATION FILED MAY 3, 1909. RENEWED FEB. 26, 1917.

1,221,397.

Patented Apr. 3, 1917.

Fig. 3.



Fig. 4.



Fig. 1.



Fig. 2.



Witnesses

A. G. Hague.  
W. A. Loftus.

Inventor

E. L. Watrous  
by Dwight Lane, atty.

# UNITED STATES PATENT OFFICE.

EDWARD L. WATROUS, OF DES MOINES, IOWA, ASSIGNOR TO E. L. WATROUS  
GALVANIZING COMPANY, A CORPORATION OF SOUTH DAKOTA.

## METHOD OF METAL-PLATING.

1,221,397.

Specification of Letters Patent.

Patented Apr. 3, 1917.

Application filed May 3, 1909, Serial No. 493,584. Renewed February 28, 1917. Serial No. 151,151.

*To all whom it may concern:*

Be it known that I, EDWARD L. WATROUS, a citizen of the United States, residing at Des Moines, in the county of Polk and State 5 of Iowa, have invented certain new and useful Improvements in Methods of Metal-Plating, of which the following is a specification.

The object of my invention is to provide 10 an improved method of plating metal such as iron with non-corrosive metal such as zinc in a smooth and uniform manner so that articles such as bolts and nuts may be thus plated and the plating material thus applied 15 will not interfere with the accurate fitting of the nuts on the bolts.

My invention consists in the arrangement 20 and combination of the various steps of the process by which the objects contemplated are attained.

In the accompanying drawings, I have 25 illustrated one form of apparatus by which the method may be carried out.

Figure 1 shows a top or plan view of a 30 furnace for melting zinc and a receptacle therein to contain articles to be plated.

Fig. 2 shows a side elevation of the furnace.

Fig. 3 shows a top or plan view of a 35 vice for applying centrifugal action to the receptacle containing articles to be coated, and—

Fig. 4 shows a central sectional view of same.

The reference numeral 10 indicates the 40 walls of a furnace, and arranged within the walls is a tank 11 in which the zinc to be melted is placed. The receptacle for containing the articles to be coated is indicated by the numeral 12 and is provided with 45 perforated sides. It also has at its top two handles 13. A rod 14 is provided to rest on top of the furnace walls and to extend through the handles 13 to support the vessel 12 in the melted zinc. The device for applying a centrifugal action to the vessel for containing articles to be plated comprises a base 15 having a stationary shield 16 thereon open at its top and bottom and widest at its 50 bottom. Arranged within this shield is a rotatable support 17 having a frame 18 mounted thereon and designed to receive and support the vessel 12. Beneath the support 17 is a number of gas jets 19 for heating the supports.

In carrying out my improved method, I first place in the receptacle of the furnace a quantity of zinc or other plating material and by applying the heat of the furnace reduce same to a melted condition. I then 55 place the articles to be coated such, for instance, as bolts, nuts, and screws in the vessel 12. This vessel is then supported in the furnace with the articles to be coated immersed in the melted zinc. The articles are 60 allowed to remain in the melted zinc and the zinc is heated to such a temperature that the pores of the metal to be plated will open up and the plating metal will enter the pores to such an extent that the coating material will 65 become homogeneous with the surface metal of the article to be coated. I then bodily remove the vessel containing the articles to be coated and instantly place same upon the rotatable support 17 which has been 70 previously heated by means of the gas jets and which is maintained at a high temperature by the gas jets. I then cause the support 17 to be rapidly rotated with the result that the 75 centrifugal action will cause all of the superfluous plating material on the articles to be coated to be discharged outwardly through the perforated sides of the vessel, thus leaving upon the articles to be coated only so 80 much of the coating material as has become 85 homogeneous with the article to be coated and leaving upon the article to be coated a uniform layer or coating of zinc which will 90 not chip or break off and which will be so uniform in thickness that articles such as nuts and bolts may be thus treated and afterward screwed together without affecting the accurate fitting of the threads.

In carrying out the process it is desirable 95 that the vessel containing the articles to be coated be transferred quickly from the furnace in which they are treated to the zinc bath to the machine in which the centrifugal action is applied. For, if the articles to be treated become chilled during the transfer 100 or during the time they are being placed in the centrifugal machine, the coating will become hardened either wholly or in part and thus prevent the superfluous coating material from being discharged. It is also desirable 105 that the rotatable plate on which the vessel containing the articles to be coated is placed be heated in such a manner as to prevent chilling during the time the centrifugal action is being applied.

I claim:—

1. The method of treating metal articles, which consists in placing the articles loosely in a perforated receptacle, then immersing the receptacle containing the articles in a bath of molten zinc by supporting said receptacle in a furnace containing said molten zinc and permitting the articles to remain in the molten zinc until the zinc alloys with the surface metal of the articles, then bodily removing the receptacle containing the articles and instantly subjecting it to centrifugal action, meanwhile maintaining the zinc in a molten state by applying heat thereto, where-  
15 by the excess zinc is thrown off, and a smooth, uniform galvanization is effected.
2. The method of treating small iron ar-  
20 ticles of complex form which consists in placing said articles loosely in a receptacle provided with perforated sides, then immersing the articles while thus supported in a bath of molten zinc by supporting the receptacle in which the articles are contained in a furnace containing the molten zinc, and then  
25 heating and allowing the articles to remain until the zinc alloys with the surface metal of the articles, subsequently placing the receptacle and articles upon a rotatable sup-  
30 port, while simultaneously heating the ar-  
ticles uniformly throughout and subjecting the receptacle and its contents to a centrifugal action whereby all excess zinc will be thrown off and a smooth uniform covering produced on the articles.
- 35 3. The method of galvanizing small ar-  
ticles which consists in placing the articles loosely in a perforated receptacle, then im-

mersing said receptacle in a bath of molten zinc until the zinc alloys with the surface metal of the articles, then bodily removing 40 the receptacle containing the articles and immediately subjecting it to rapid centrifugal action without removing the articles therefrom until the excess zinc is thrown off and a smooth, uniform galvanization is effected. 45

4. The method of galvanizing small ar-  
ticles which consists in placing said articles in a perforated receptacle, in immersing said receptacle together with the articles in molten zinc until a thorough surface alloy 50 between the articles and the zinc takes place, in then removing and subjecting the articles and receptacle together to centrifugal action, whereby from the beginning to the end of the process of galvanizing, the articles are 55 maintained in the same receptacle and therefore can never come in contact with a sur-  
face cooler than themselves.

5. The method of treating metal articles which consists in placing the articles loosely 60 in a perforated receptacle, then immersing said receptacle in a bath of molten metal until said metal alloys with the surface metal of the articles, then bodily removing the receptacle containing the articles and immedi-  
ately subjecting it to rapid centrifugal ac-  
tion without removing the articles therefrom until the excess coating metal is thrown off and a smooth uniform coating is effected. 65

Des Moines, Iowa, April 9, 1909.  
EDWARD L. WATROUS.

Witnesses:

MILDRED B. GOLDIZEN,  
NELLIE M. TAYLOR.